

2,908,573

## PHOTOGRAPHIC COLOR COUPLERS CONTAINING MONO-n-ALKYL GROUPS

Walter M. Bush, Ilmari F. Salminen, and John R. Thirlfle, Rochester, N.Y., assignors to Eastman Kodak Company, Rochester, N.Y., a corporation of New Jersey

No Drawing. Application July 25, 1956  
Serial No. 599,896

9 Claims. (Cl. 96—100)

This invention relates to color photography and particularly to photographic color formers containing normal alkyl groups.

The formation of colored photographic images by coupling the development product of primary aromatic amino developing agents with color-forming or coupling compounds is well known. In these processes the subtractive process of color formation is ordinarily used and the image dyes are of the complementary primary colors cyan, magenta and yellow. The couplers used to produce these dyes generally contain color-forming groups of the phenolic hydroxyl, pyrazolone or benzoyl acetamide classes. These groups render the coupler capable of coupling with the oxidation product of the primary aromatic amino developing agent on photographic development.

When these color-forming compounds are incorporated in the silver halide emulsion layer prior to photographic development, they usually contain groups which render them non-diffusing in the emulsion layer. Tertiary amyl and other branched chain alkyl radicals have been used for this purpose and normal alkyl radicals attached to nitrogen or oxygen atoms have also been employed.

One of the disadvantages of the tertiary amyl and other branched chain alkyl radicals in color-forming compounds is that they raise the melting point of the coupler and thus increase its tendency to crystallize in the emulsion. They are also usually of limited solubility in organic solvents and the amount which can be incorporated in the emulsion layer is therefore limited.

It is therefore an object of the present invention to provide novel photographic coupler compounds for incorporation in silver halide emulsion layers. A further object is to provide coupler compounds having lower melting points than those hitherto employed and therefore having lower tendency to crystallize in the emulsion. A still further object is to provide coupler compounds which are more soluble in organic solvents than those hitherto employed, thus permitting higher concentrations of coupler to be used and higher dye densities to be obtained. A still further object is to provide coupler compounds which have lower diffusivity in the emulsion layer than those previously employed. Other objects will appear from the following description of our invention.

These objects are accomplished according to our invention by the use of couplers containing a single normal alkyl radical attached to an aryl radical, especially to a phenoxy acylamino radical. Couplers which we propose to use have one of the following structures:



in which Z is a phenolic hydroxyl, pyrazolone or benzoyl acetamide group which is capable of coupling with the

oxidation product of a primary aromatic amino developing agent, and which includes one or more aryl radicals, R is hydrogen or an ethyl radical, R' is a normal alkyl radical containing from 7 to 15 carbon atoms, for example, a normal heptyl, normal octyl, normal nonyl, normal tridecyl or normal pentadecyl radical in the ortho, meta or para position, and n is 0, 1 or 2.

More specifically, the classes of color-forming compounds which we employ have one of the following structures:

(II)



(III)



(IV)



in which one X is hydrogen and the other X is



and in which R, R' and n are the same as above.

Typical couplers which we may use according to our invention are as follows:

### CYAN

(1)



(1a)



(2)



(3)





## MAGENTA



## YELLOW



The couplers of our invention were prepared as follows:

10 No. 1:  $\alpha$ -(3-n-pentadecylphenoxy)acetic acid.—A mixture of 25.2 g. (0.1 mole) of 3-n-pentadecylphenol, 6.0 g. (0.11 mole) of potassium hydroxide pellets, and 150 cc. of xylene was stirred and boiled until 75 cc. of wet xylene had been collected. An additional 100 cc. of xylene was 15 added and the process continued until a total of 110 cc. had been collected. To the solution was added 11.6 g. (0.1 mole) of sodium chloroacetate, and stirring and refluxing were continued for 3 hours. The mixture was cooled to room temperature and acidified with 25 cc. of 20 hydrochloric acid and 50 cc. of ice water. The solid was collected, washed, and then dissolved in 600 cc. of ether, from which it separated on concentration. Crystallization from a mixture of ligroin and benzene gave a material which melted at 99–100° C.

25  $\alpha$ -(3-n-pentadecylphenoxy)acetyl chloride.—A mixture of  $\alpha$ -(3-n-pentadecylphenoxy)acetic acid and an excess of thionyl chloride was heated at 50–56° for 4 hours. The excess thionyl chloride was removed under vacuum and the solid residue was used directly in the next step.

30 2,4-dichloro-3-methyl-6-[ $\alpha$ -(3-n-pentadecylphenoxy)-acetamido]phenol.—To a mixture of 2.3 g. (0.01 mole) of 6-amino-2,4-dichloro-3-methylphenol hydrochloride and 2.5 g. (0.03 mole) of anhydrous sodium acetate in 45 cc. of 90% acetic acid, was added 3.8 g. (0.01 mole) 35 of  $\alpha$ -(3-pentadecylphenoxy)acetyl chloride. The reaction was permitted to continue spontaneously for seven minutes; then the mixture was heated externally to 53°. When the mixture had cooled to 40°, 50 cc. of water was 40 added and the solid was collected and washed with water followed by a little methanol. The product was crystallized from a mixture of ether-petroleum ether giving a yield of 3.2 g., which melted at 122–4°. Recrystallization from acetonitrile raises the melting point to 129–130° C.

45 Couplers Nos. 2 and 3 were made similarly to coupler No. 1 using respectively  $\alpha$ -(3-n-pentadecylphenoxy)-n-butyryl chloride and  $\gamma$ -(3-n-pentadecylphenoxy)-n-butyryl chloride instead of 3-n-pentadecylphenoxy acetyl chloride.

50 Coupler No. 4 was made in the same way as coupler No. 1 of U.S. Patent 2,474,293 using 3-n-pentadecylphenol instead of 2,4-di-tert.-amylphenol.

Coupler No. 5 was made as follows:

2-caprylylamido-5-nitrophenol.—To a solution of 15.4 g. (0.1 mole) of 2-amino-5-nitrophenol, and 26 g. (0.2 55 mole) of quinoline in 150 cc. of dioxane was added, with stirring at 25° C., a solution of 17.8 g. (0.11 mole) of octanoyl chloride in 50 cc. of dioxane. The temperature rose rapidly to 35° C. and a clear amber reaction mixture resulted. This mixture was left to stand overnight at room temperature, after which time it was poured into 600 cc. of dilute hydrochloric acid. The solid product was filtered off, dried, and recrystallized from 300 cc. of toluene.

5-amino-2-caprylylamidophenol.—In a 500 cc. low 65 pressure reduction bottle was placed a solution of 7 g. (0.025 mole) of 2-caprylylamido-5-nitrophenol in 100 cc. of dioxane. To this solution was added one part of Raney nickel catalyst, and the bottle was placed on the Parr hydrogenation apparatus. The hydrogen pressure 70 was brought up to 50 lb. and shaking commenced. The reduction was complete after approximately one hour. The mixture was filtered, and the solution of the amine was used without isolation.

2-caprylylamido-5-[ $\alpha$ -(3-n-pentadecylphenoxy)-n-butyryl-amido]phenol.— $\alpha$ -(3-n-pentadecylphenoxy)-butyryl chlo-

ride was prepared in the same way as  $\alpha$ -(3-pentadecylphenoxy)acetyl chloride except that ethyl  $\alpha$ -bromobutyrate, followed by saponification, was used instead of sodium chloroacetate. To a solution of 6.25 g. (0.025 mole) of 5-amino-2-caprylamidophenol and 6.45 g. (0.05 mole) of quinoline in 150 cc. of dioxane was added, with stirring at 26° C., a solution of 10.2 g. (0.025 mole) of  $\alpha$ -(3-pentadecylphenoxy)-n-butyryl chloride in 40 cc. of dioxane. The temperature rose rapidly to 31° C. and a clear reaction mixture resulted. This mixture was stirred for one hour at room temperature, and then poured into 1 l. of dilute hydrochloric acid. The solid product was filtered off, dried, and recrystallized five times from approximately 10 parts of acetonitrile to give a compound melting at 85–86° C.

Coupler No. 6 was made in the same way as coupler No. 9 of U.S. Patent 2,600,788 using  $\alpha$ -(3-n-pentadecylphenoxy)-n-butyryl chloride instead of  $\beta$ -(2,4-di-tert-amylphenoxy)propionyl chloride.

Coupler No. 7 was made in the same way as coupler No. 7 of U.S. Patent 2,600,788 using  $\alpha$ -(3-n-pentadecylphenoxy)-n-butyryl chloride instead of 2,4-di-tert-amylphenoxy acetyl chloride.

Coupler No. 8 was made in the same way as coupler No. 6 using 2,4,5-trichloroaniline instead of 2,4,6-trichloroaniline.

Coupler No. 9 was made in the same way as coupler No. 7 using 2,4,5-trichloroaniline instead of 2,4,6-trichloroaniline.

Coupler No. 10 was prepared as follows:

$\alpha$ -(*m*-Nitrobenzoyl)-2-methoxyacetanilide.—To a refluxing mixture of 22 g. (0.093 mole) of ethyl  $\alpha$ -(*m*-nitrobenzoyl)-acetate (Bülow and Hailer, Ber., 35, 915 (1902)) in 150 ml. of histological xylene was added in one portion 11 g. (.09 mole) of *o*-anisidine. The mixture was heated at the reflux temperature (oil bath at 145–55° C.) for two hours under a steam-jacketed still-head, which permitted the removal of the alcohol-xylene azeotrope. The product which separated from the cooled reaction mixture was filtered and sucked dry on a Buchner funnel; the yield of yellow product was 24 g. (82%), M.P. 166–7° C.

$\alpha$ -(*m*-Aminobenzoyl)-2-methoxyacetanilide.—In a 5-liter, three-necked flask, equipped with stirrer, reflux condenser and addition tube, were placed 104 g. of technical-grade sodium sulfide (0.8 mole) and 200 ml. of water. The mixture was stirred gently on a steam bath until solution was complete, and 3200 ml. of ethyl alcohol were added. The mixture was boiled and 126 g. (0.4 mole) of  $\alpha$ -(*m*-nitrobenzoyl)-2-methoxyacetanilide were added portionwise over a period of fifteen minutes with good stirring. The brown reaction mixture was heated at the boiling point for one-half hour and poured on about an equal volume of ice. To the cold solution was added 212 g. (4 moles) of solid ammonium chloride. The mixture was stirred manually until the ammonium chloride was dissolved, and allowed to stand for forty minutes. The product was filtered by suction and washed on the funnel with several liters of water, until the washings were colorless. The pale-yellow product was dissolved in 1600 ml. of boiling alcohol and 100 ml. of hot water added. A small amount of Darco was added, and the solution was filtered while hot. The cooled filtrate yielded 89.1 g. (78.5%) of fluffy yellow product, M.P. 139.5–40° C.

$\alpha$ -(3-[ $\alpha$ -(2,4-di-tert-amylphenoxy)acetamido]benzoyl)-2-methoxyacetanilide.—In a 500-cc. three-necked flask, provided with a stirrer and thermometer, were placed 300 cc. of 90 percent acetic acid and 30 g. (0.36 mole) of anhydrous sodium acetate. To this solution, at room temperature, was added 32.0 g. (0.1 mole) of  $\alpha$ -(*m*-aminobenzoyl)-2-methoxyacetanilide hydrochloride, an easily stirrable mixture resulting as the temperature dropped 2° C. After this mixture had been stirred for one-half hour, 37 g. (0.19 mole) of  $\alpha$ -(3-n-pentadecylphenoxy)-n-butyryl chloride was added during

approximately one-half minute. The reaction mixture became much thinner, but failed to clear up as the temperature rose from 25.5° C. to 33.5° C.; color was a pink-gray. Following one and one-half hours of stirring, the mixture was diluted dropwise over a period of one-half hour with 30 cc. of water and seeded with coupler. Further stirring overnight caused separation of product as a finely divided white mass.

The reaction mixture was drowned with stirring during fifteen minutes in 600 cc. of water, the product separating in white granules. Stirring was continued for forty-five minutes and the mixture filtered readily through a 5-inch Buchner funnel. The white solid was washed on the funnel with 2 liters of water, not over 20° C. Immediately, when the cake was no longer covered by water, it shrank in a characteristic manner away from the edge of the funnel as though threatening to become gummy. This change failed to occur as the cake was sucked and pressed thoroughly. The solid, which could be broken up easily, was air-dried, 60 g. being obtained; it had an indistinct melting range, starting at about 95° C.

Twelve hundred cc. of cyclohexane was heated to a boil on the steam bath and the 60 g. of crude product dissolved therein, forming a pink solution. It was treated with 2 g. of Darco and the solution filtered hot through 2 g. of Darco on a 4-inch Buchner funnel. Clear filtrate was only slightly less colored than prior to the Darco treatment. The coupler was permitted to crystallize undisturbed overnight. It was filtered readily, washed on the

funnel with three 100-cc. portions of fresh cyclohexane. The yield was 47 g. (82% of the theoretical amount) of white coupler, which melted at 126–127° C.

Coupler No. 11 was prepared as follows:

$\alpha$ -Benzoyl-2-methoxy-5-nitroacetanilide.—In a 250-ml. round bottom flask equipped with a partial condensing stillhead were placed 100 ml. of histological xylene and 16.8 grams (0.1 mole) of 4-nitro-2-aminoanisole (Ber. 13, 389). The mixture was brought to a boil and 19.2 grams (0.1 mole) of ethyl benzoylacetate was added all at once. After refluxing 2 hours, about 3–5 ml. of ethyl alcohol had been collected. The yellow solution was filtered hot and allowed to cool to room temperature. The yellow solid which separated was filtered, washed with 50 ml. of xylene, and finally with 100 ml. of petroleum ether. A crude yield of 26 grams (83 percent) was obtained which melted at 170–175° C. On recrystallization from 18 parts of glacial acetic acid, 22.4 grams (71 percent) of fine light yellow needles, M.P. 177–179° C., was obtained.

$\alpha$ -Benzoyl-5-amino-2-methoxyacetanilide.—In a Parr hydrogenation bottle were placed 16 grams (0.051 mole) of  $\alpha$ -benzoyl-2-methoxy-5-nitroacetanilide, 250 ml. of absolute ethyl alcohol, and 2–5 grams of Raney nickel. The reaction mixture was shaken under 2–3 atmospheres of hydrogen overnight at room temperature. The nickel was removed by filtration and the filtrate cooled in an ice bath. The light yellow solid was filtered, washed with 50 ml. of cold methyl alcohol, and dried. The yield was 13 grams (90 percent) of a solid which melted at 108–110° C.

3-benzoylacetamino-4-methoxy-(2',4'-di-tert-amylphenoxy)-acetanilide.—In a 250-ml. Erlenmeyer flask were placed 5.68 grams (0.02 mole) of  $\alpha$ -benzoyl-5-amino-2-methoxyacetanilide, 2 grams (0.02+ mole) of anhydrous sodium acetate, and 100 ml. of glacial acetic acid. With good stirring 6.2 grams (0.02 mole) of  $\alpha$ -(3-n-pentadecylphenoxy)-n-butyryl chloride in 25 ml. of glacial acetic acid was added all at once. The reaction mixture was stirred 1 hour at room temperature and 1/2 hour at 60° C. After cooling to room temperature, the reaction mixture was poured with vigorous stirring into 1 liter of cold water. The moist solid was filtered, washed with cold water, sucked as dry as possible, and recrystallized from 200 ml. of denatured alcohol. The yield was 7.5 grams (67 percent) of a tan powder which

melted at 124–126° C. Recrystallization from 200 ml. of alcohol gave 6.2 grams (55%) of a product which melted at 132–134° C.

Coupler 1a was prepared as follows:

p-n-Octylphenol was prepared as described by Sandulesco and Girard, Bull. Soc. Chim., 47, 1300 (1930), and was converted to p-n-octylphenoxyacetic acid (M.P. 92-3°) by reaction of the phenol sodium salt with sodium chloroacetate. The acid chloride (0.540°) was prepared from the acid by reaction with thionyl chloride. Reaction of the acid chloride with the coupler amine (6-amino-2,4-dichloro-3-methylphenol) in the presence of a sodium acetate-acetic acid buffer gave the coupler, melting at 141-2°. Recrystallization from glacial acetic acid raised the melting point to 141.5-142°.

The lowering of the melting points of the couplers by the normal alkyl group, compared with the corresponding compound containing a tertiary or branch chain group is shown in the following table:

|                                     | M.P., ° C. |
|-------------------------------------|------------|
| Coupler No. 1a                      | 141.5-142  |
| Same coupler with tert. octyl group | 149-152    |

The following example illustrates the incorporation of our couplers in a silver halide emulsion.

### Example

One gram of coupler No. 1 was dissolved by warming by 2 cc. of tri-o-cresyl phosphate. This solution was combined with a mixture of 50 cc. of 10% gelatin solution, 5 cc. of 5% Alkanol B solution and 30 cc. of distilled water, and the whole passed through a colloid mill several times. To the resulting dispersion was added 20 cc. of a gelatino-silver halide emulsion and the mixture was coated in the usual manner.

After exposure, this emulsion was developed in the following solution:

|                                   | Grams |
|-----------------------------------|-------|
| 2-amino-5-diethylaminotoluene HCl | 2     |
| Sodium sulfite (desiccated)       | 2     |
| Sodium carbonate, monohydrate     | 20    |
| Potassium bromide                 | 2     |
| Water to 1 liter.                 |       |

After development, the emulsion was fixed in the usual acid-alum fixing bath, washed, and the silver removed by successive treatments in ferricyanide-bromide solution and hypo.

The improved solubility of our couplers is illustrated by the fact that 1 gram of coupler No. 1 dissolves in 2 cc. of the coupler solvent di-n-butyl phthalate at 125° C., whereas the corresponding coupler containing a tertiary alkyl group could be dissolved to the extent of 1 gram in 2 cc. of the coupler solvent only when the temperature was raised to 142° C. Similarly, 1 gram of coupler No. 8 dissolves in 1 cc. of the coupler solvent tri-o-cresyl phosphate at 54° C. while the corresponding coupler containing a tertiary alkyl group could be dissolved to the extent of 1 gram in 1 cc. of the coupler solvent only by raising the temperature to 115° C. Couplers containing the monoalkyl phenoxy groups are therefore more soluble than those containing tertiary alkyl groups. These higher solubilities permit higher concentrations of couplers in coupler solvent to be used in the coatings and results in higher dye densities in the emulsion coatings.

In addition to incorporating the coupler in the emulsion as described above, our couplers may also advantageously be incorporated in the emulsion as described in Fierke and Chechak U.S. Patent 2,801,171. This method involves the preparation of low coupler-to-coupler-solvent ratio dispersion. The coupler is first dissolved in either a low-boiling water-insoluble organic solvent or an appreciably water-soluble organic solvent with or without a high-boiling water-insoluble organic solvent, the solution dispersed in gelatin and the dispersion chilled and

set and at least 90% of the water and substantially all of the low-boiling water-insoluble solvent or the appreciably water-soluble organic solvent removed. When emulsions made in this way are exposed and color developed, the dye density is usually higher than that obtained from the emulsions made in the manner described in the examples above.

In addition to being incorporated in gelatino-silver halide emulsion layers, our couplers may be incorporated in silver halide layers in which the emulsion carrier is an organic acid ester of cellulose or a synthetic resin. The support may be a transparent medium such as glass or cellulose ester or a non-transparent reflecting medium such as paper or an opaque cellulose ester. The emulsion may be coated as a single layer on the support or superposed layers may be coated on one or both sides of the support. The superposed layers may be differentially sensitized to form a natural color element in the known manner.

The examples and compounds set forth in the present specification are illustrative only and it is to be understood that our invention is to be taken as limited only by the scope of the appended claims.

We claim:

1. A color-forming photographic emulsion containing a color-forming compound of low diffusivity, comprising a gelatino-silver halide emulsion containing a color-forming compound selected from the class consisting of compounds having the structure



and



where Z is a color-forming group including an aryl radical, capable of coupling with the oxidation products of a primary aromatic amino developing agent, selected from the class consisting of phenolic hydroxyl, pyrazolone and benzoylacetamide groups, R is selected from the class consisting of hydrogen and an ethyl radical, R' is a normal alkyl radical containing from 7 to 15 carbon atoms in a position selected from the class consisting of ortho, meta and para, and n is from 0 to 2.

2. A color-forming photographic emulsion containing a color-forming compound of low diffusivity, comprising a gelatino-silver halide emulsion containing a color-forming compound having the structure



where R is selected from the class consisting of hydrogen and an ethyl radical, R' is a normal alkyl radical containing from 7 to 15 carbon atoms, and n is from 0 to 2.

3. A color-forming photographic emulsion containing a color-forming compound of low diffusivity, comprising a gelatino-silver halide emulsion containing a color-forming compound having the structure



where  $R'$  is a normal alkyl radical containing from 7 to 15 carbon atoms.

4. A color-forming photographic emulsion containing a color-forming compound of low diffusivity, comprising

9

a gelatino-silver halide emulsion containing a color-forming compound having the structure



where one X is hydrogen and the other X is



and R' is a normal alkyl radical containing from 7 to 15 carbon atoms.

5. A color-forming photographic emulsion containing a color-forming compound of low diffusivity, comprising a gelatino-silver halide emulsion containing a color-forming compound having the structure



6. A color-forming photographic emulsion containing a color-forming compound of low diffusivity, comprising a gelatino-silver halide emulsion containing a color-forming compound having the structure



7. A color-forming photographic emulsion containing a color-forming compound of low diffusivity, comprising a gelatino-silver halide emulsion containing a color-forming compound having the structure

2,908,573

10



5

10

15

8. A color-forming photographic emulsion containing a color-forming compound of low diffusivity, comprising a gelatino-silver halide emulsion containing a color-forming compound having the structure



20

25

30

35

40

45

9. A color-forming photographic emulsion containing a color-forming compound of low diffusivity, comprising a gelatino-silver halide emulsion containing a color-forming compound having the structure



References Cited in the file of this patent

UNITED STATES PATENTS

|           |                 |                |
|-----------|-----------------|----------------|
| 2,186,849 | Wilmanns et al. | Jan. 9, 1940   |
| 2,425,503 | Bavley          | Aug. 12, 1947  |
| 2,652,329 | McCrossen       | Sept. 15, 1953 |
| 2,704,711 | Hanson          | Mar. 22, 1955  |
| 2,721,798 | Loria et al.    | Oct. 25, 1955  |
| 2,808,329 | Whitmore        | Oct. 1, 1957   |

UNITED STATES PATENT OFFICE  
Certificate of Correction

Patent No. 2,908,573

October 13, 1959

Walter M. Bush et al.

It is hereby certified that error appears in the printed specification of the above numbered patent requiring correction and that the said Letters Patent should read as corrected below.

Column 2, lines 42 to 47, the formula should appear as shown below instead of as in the patent:



column 3, lines 33 to 36 inclusive, right-hand portion of the formula should appear as shown below instead of as in the patent:



column 7, line 9, for "( $_{0.5}^{40^\circ}$ )" read —( $_{0.5}^{140^\circ}$ )—.

Signed and sealed this 7th day of June 1960.

[SEAL]

Attest:

KARL H. AXLINE,  
*Attesting Officer.*

ROBERT C. WATSON,  
*Commissioner of Patents.*